

## UNITED STATES PATENT OFFICE

2,049,927

METHOD OF MAKING BRITTLE  
METALS OR ALLOYS

Walter E. Remmers, Western Springs, Ill., assignor to Western Electric Company, Incorporated, New York, N. Y., a corporation of New York

No Drawing. Application May 10, 1934,  
Serial No. 724,912

8 Claims. (Cl. 75—82)

This invention relates to a method of making brittle metals or alloys and more particularly to a method of making brittle nickel-iron alloys.

In the manufacture of brittle alloys which are 5 to be pulverized for the purpose of forming the particles into compressed magnetic cores, it has been difficult to obtain the correct degree of brittleness of the alloys for reducing the ingots cast from the alloys into small particles.

10 An object of the invention is to provide an effective and simple method of making brittle alloys.

In accordance with one embodiment of the invention, the alloys are first oxidized to a readily 15 determinable degree, after which a predetermined amount of a deoxidizing agent is added to obtain the desired degree of brittleness.

Magnetic cores, such as used for loading coils 20 in telephone communicating systems, are usually made from insulated and compressed magnetic particles, which may be of a fineness varying in size from particles that will pass through a 100 mesh sieve to particles that will pass through a 300 mesh sieve. In order to obtain these fine 25 particles, the magnetic materials must be embrittled so that when they are cast into ingots and hot rolled, the material will break up into relatively small lumps and the brittleness of the material is also a factor in grinding these lumps 30 into a fine powder. The hot rolling of the ingots is usually accomplished in a mill which has a fixed number of passes. If, for instance, a mill is used having thirteen passes, the ingot must have such a degree of brittleness that it will not 35 crack up appreciably prior to the thirteenth pass and break up into relatively small lumps at the thirteenth pass from which it is dropped into a quenching tank. Considerable difficulty has been experienced in obtaining the proper degree of 40 brittleness to break the material into relatively small lumps and cause it to pulverize without requiring an undue amount of grinding.

One of the most common materials used for 45 magnetic dust cores is a nickel-iron alloy in which the nickel may vary from 45% to more than 83% of the alloy. Even though these materials, that is the nickel and iron, are relatively pure, the nickel usually contains some sulphur and the iron contains fractional percentages of carbon, manganese, silicon, sulphur, phosphorus, and some occluded gases, such as carbon monoxide and hydrogen. The sulphur content of the iron is usually quite uniform and ranges from .009% to .012% or over. The nickel and iron are melted 50 together under a covering of lime and fluor-

spar slag to which iron oxides are added either in the form of  $Fe_2O_3$  or  $Fe_3O_4$ . The iron oxides tend to oxidize the impurities and gases in the molten alloy and during this oxidation the brittleness of the alloy changes from a state in which it is too ductile or tough to a state in which it is too brittle. The quantity of oxides which must be added varies with the amount and kind of impurities in the iron and nickel used. Obviously other methods of oxidizing the molten bath may 10 be used as the bubbling or blowing of oxygen or air through the bath.

Experience has shown that in practice there is no convenient method of determining and interrupting the process of oxidation at the point 15 of correct brittleness for the subsequent breaking up and pulverizing of the alloy. The applicant has found, however, that there is a determinable and readily recognizable point of oxidation in which the material is too brittle but 20 from which it may be readily returned to the correct degree of brittleness by the addition of a deoxidizing agent. In order to control the brittleness of the alloy, test bars which may be one inch in cross-section and five inches in length are 25 cast from time to time in an open top mold as the process of oxidation progresses. As long as the desired degree of oxidation has not been obtained, a cross-section of the test bar will disclose fissures and gas pockets, and the surface of the 30 bar will have a spew or ridge of expelled metal extending partly or wholly around the perimeter thereof. This ridge presents a rather interesting and strange phenomenon since it usually begins along the middle of one or the other of the 35 long sides of the surface and progressively travels around the perimeter, giving it the appearance of a moving worm. When the oxidation has progressed to the desired point, a cross-section of the bar is solid and the ridge no longer appears 40 on the surface of the test bar but instead the top surface of the bar is relatively flat and may be slightly concave. At this point, considerable additions of oxides to the molten metal cause but slight changes in the brittleness of the alloy. 45 The condition of the bar now indicates that the oxidation has reached a definite point, at which, however, the alloy is too brittle. The alloy may then be returned to any desired degree of brittleness by the addition of a known amount of a 50 deoxidizing agent, such as, for instance, manganese, preferably in the form of ferro-manganese. It is believed that the brittleness is a function of the sulphur content and the oxygen content or of a combination of the sulphur and oxygen 55

contents. The addition of the ferro-manganese causes the ridge to reappear on test bars cast from the alloy and for one specific purpose sufficient ferro-manganese is added to cause the ridge 5 to extend around one-half of the perimeter of the surface of a test bar. The manganese appears to control the effectiveness of the sulphur content in addition to its action as a deoxidizing agent. Of course, a greater or lesser amount 10 of the deoxidizing agent may be used to cause the ridge to extend to a greater or lesser degree around the perimeter of a test bar, depending upon the brittleness desired in the alloy. Other deoxidizing agents may be used, such as 15 aluminum, silicon, chromium, or magnesium.

In the case of a nickel-iron alloy containing 81% of nickel and the balance substantially iron, sufficient ferro-manganese is added so that the manganese constitutes from approximately .06% 20 to .11% of the alloy by weight. When this alloy is hot rolled from a temperature of about 2350° F., it is broken up into relatively small lumps with the required number of passes through the rolling mill and the lumps may then be pulverized 25 in an attrition mill and formed into magnetic cores.

It will be understood that the nature and embodiments of the invention herein described are merely convenient and useful forms of the invention and that many changes and modifications may be made therein without departing 30 from the spirit and scope of the invention.

What is claimed is:

1. A method of making a brittle nickel-iron alloy, which comprises adding oxides to the molten alloy to reduce its ductility, testing the alloy 35 progressively as said ingredients are added until a cast specimen of the alloy reaches a predetermined characteristic state having a substantially flat surface, and adding an amount of a deoxidizing agent to produce the desired brittleness insufficient to completely reduce the melt.

2. A method of making a brittle nickel-iron alloy, which comprises adding metallic oxides to 45 the molten alloy, progressively casting test specimens of the alloy as said oxides are added until a specimen is obtained which is substantially devoid of a peripheral ridge, and adding a predetermined amount of a deoxidizing agent insufficient 50 to completely reduce the melt.

3. A method of making a brittle nickel-iron alloy, which comprises adding metallic oxides to the molten alloy, progressively casting test specimens of the alloy as said oxides are added until

a specimen is obtained which is substantially devoid of a peripheral ridge, and adding a definite amount of manganese, insufficient to completely reduce the melt.

4. A method of making a brittle nickel-iron 5 alloy, which comprises adding oxidizing materials to the molten alloy, progressively casting test specimens of the alloy as said materials are added until a specimen is obtained having a substantially flat surface, and adding an amount of a deoxidizing agent to produce the desired brittleness.

5. A method of making a brittle nickel-iron alloy, which comprises adding oxidizing materials 10 to the molten alloy, progressively casting test specimens of the alloy as said materials are added until a specimen is obtained being substantially devoid of a peripheral ridge, adding a deoxidizing agent until a specimen is obtained having a predetermined length of peripheral ridge, casting 15 the alloy into ingots, and hot rolling the ingots to break them into fragments.

6. A method of making a brittle alloy, which comprises alloying iron containing sulphur and other impurities with nickel, oxidizing the alloy 20 to embrittle the alloy beyond the extent desired for comminuting the material, progressively casting test specimens of the alloy until a specimen is obtained being substantially devoid of a peripheral ridge and adding a measured amount 25 of a deoxidizing agent selected from the group of manganese, aluminum, silicon, chromium, and magnesium to obtain the desired degree of brittleness.

7. A method of making a brittle alloy, which 30 comprises alloying iron and nickel containing oxidizable impurities, oxidizing the alloy to embrittle the alloy beyond the extent desired for comminuting the material, progressively casting test specimens of the alloy until a specimen is obtained being substantially devoid of the peripheral ridge, and adding a measured amount of a deoxidizing agent to obtain the desired degree of brittleness.

8. The steps in the method of embrittling a 45 nickel-iron alloy which comprise adding metallic oxides to the molten alloy until a predetermined characteristic state is reached in which a cast specimen of the alloy is substantially devoid of a peripheral ridge, and adding a predetermined 50 amount of a deoxidizing agent insufficient to completely reduce the melt.

WALTER E. REMMERS.